

1

3,001,948

## SYNTHETIC DETERGENT BAR

Everett Clippinger, San Rafael, Calif., assignor to California Research Corporation, San Francisco, Calif., a corporation of Delaware  
No Drawing. Filed Nov. 26, 1957, Ser. No. 700,250  
4 Claims. (Cl. 252—152)

The present invention relates to molded or shaped synthetic detergent compositions of any desired shape or form and to a process for the preparation thereof. More particularly, the invention has to do with the preparation of a detergent bar for toilet and bath use containing as the essential detergent material a special kind of synthetic surfactant, the particles of which can unexpectedly be compacted or pressed into a lastingly sturdy mass or body.

Much effort has been, and is being, expended in the art of synthetic detergents on the search for a superior detergent bar, and for the improvement of existing non-soap detergent bars. As is known, synthetic detergents are superior in certain respects to soap; for example, their efficiency is not impaired in hard or salt water. Formulations of soap and certain synthetic detergents have been proposed but without the hoped-for superiority, and indeed suffer from certain disadvantages, such as poor lather, and poor solubility characteristics. On the other hand, it is desirable that non-soap detergent bars be like soap in other respects. It is thus desirable that synthetic non-soap detergent bars have low hygroscopicity, proper rate of solution, good lathering characteristics, a pleasant feeling on contact with the skin, freedom from stickiness, harmlessness to the human body, and ability to be produced in conventional soap-making equipment.

An essential feature in the preparation of a synthetic detergent bar is that the surfactant employed in its preparation be capable of being formed, i.e., milled, shaped or molded, into a stable, lastingly sturdy, non-brittle bar. Accordingly, in order to prepare a bar with the desired characteristics, it has heretofore been found necessary to incorporate with the surfactant various organic binders or plasticizers capable of modifying the physical characteristics of the detergent mass and of binding together the detergent particles into a compact cohesive bar or cake. As examples of binding agents there can be mentioned starches, polyhydric alcohols partially esterified with saturated fatty acids, and other oleaginous materials, such as the higher alcohols, waxes and petroleum jelly.

A principal object of the present invention, therefore, is to prepare a novel detergent bar or cake without the requirement of an organic binder, the bar, moreover, having satisfactory deterging and sudsing characteristics, a proper rate of solution, good lathering characteristics, a low hygroscopicity, whereby mushing and sliming in the presence of water is at a minimum, and one which gives a pleasant feeling to the user during and after use.

In accordance with the invention there are contemplated detergent bar compositions based on normally plastic synthetic detergent material of ammonium detergent salts of alkylsulfonic acids, and, in association therewith, a second metal detergent salt of alkylsulfonic acids, the alkyl groups in both instances being primary straight-chain radicals of about 8, preferably 10, to 20 carbon atoms, the detergent material having an average carbon content of 12 to 16 carbon atoms. Ordinarily, the composition contains water in an amount by a weight, based on the detergent material, of about 1 to 10%, usually around 5 to 8%.

In my copending application Serial No. 698,915, filed November 26, 1957, there are described and claimed synthetic detergent bars based on ammonium n-alkyl-

2

sulfonates. However, in order to prepare a cake or bar possessing satisfactory characteristics in accordance with the aforesaid application, the sulfonates are required to be derived from a rather narrow class of olefins. It has now unexpectedly been found that ammonium n-alkylsulfonates of a broader class can satisfactorily be solidified, milled and molded into an effective detergent bar by the incorporation with the ammonium n-alkylsulfonate mixture of a second metal n-alkylsulfonate detergent salt material, the alkyl groups again being primary straight-chain radicals of 8 to 20 carbon atoms averaging 12 to 16 carbon atoms in the molecule. Inasmuch as the results achieved are due to the combination of salts of different cations, the metal salt sulfonates can be derived from a number of metals, including the alkali metals, for example, sodium and potassium; the alkaline earth metals, e.g., barium, calcium and magnesium; and other metal material, e.g., aluminum.

In general, an amount of second metal n-alkylsulfonate detergent salt is selected within about the range of 10 to 15 mol percent to 75 mol percent and higher based on total sulfonate content. For optimum results, the amount, of course, will depend on the sulfonate selected. Thus, for the alkali metal sulfonates slightly higher amounts near the top limit of the range can be selected, that is, around 75 mol percent, while with the polyvalent metal sulfonates lesser amounts will be satisfactory, that is, below about 50 mol percent. In most cases, a satisfactory mixture will consist of around 50 mol percent of the ammonium n-alkylsulfonate and 50 mol percent of the second metal n-alkylsulfonate material.

In forming the detergent material for molding, it is important that an intimate admixture of ammonium and metal sulfonate salts of the character described be effected. Accordingly, a convenient method of preparing the alkylsulfonates falling within the purview of the invention is by means of the ammonium bisulfite free radical addition to the appropriate olefins, followed by displacement of the ammonium radical by the addition of an appropriate base, e.g., sodium hydroxide, to the desired extent. In the sulfitation reaction some inorganic sulfate may be formed as a side-product, but its presence has not been found to be deleterious. Accordingly, it has been found that up to 20% by weight of the inorganic sulfate, e.g., ammonium or sodium sulfate, can be tolerated in the final composition. By the in situ formation of the sulfonates, intimate admixture of the various salts can be effected and the optimum compositions obtained.

A convenient source of the olefins for preparing the sulfonates contemplated by the invention are those that can be derived from the cracking of petroleum wax to yield a mixture primarily of 1-olefins having from about 8 to 20 carbon atoms in the molecule. It is the sulfonates of these olefins which can be blended, if necessary, to yield the desired alkylsulfonates having an average carbon content of 12 to 16 carbon atoms.

Moreover, the sulfonates contemplated by the invention are primarily and essentially those derived from 1-olefins of the specified carbon content, and are essentially of normal or straight-chain structure, although, as is known in the art, a small degree of branching may be permitted without substantial impairment of the deterging action of the material. Accordingly, characterization of the anionic portion of the sulfonate as being a primary straight-chain radical means that the sulfonate is derived essentially from normal 1-olefins in which a scattering of unsaturation in the molecule and a tolerable degree of chain branching may exist in the mixture of compounds without its adversely affecting the deterging action of the materials.

As above suggested, important criteria of a satisfactory

bar are subjective or organoleptic in nature and are based largely on experience derived from the properties possessed by the conventional soap bar. Thus, the over-all nature of the bar, such as waxy appearance and color, odor, impressions on touch, such as stickiness; and feeling by the user during use and after use are not so much determinable by objective standards as they are by averaged personal reactions.

Certain other characteristics of a bar however, lend themselves readily to objective evaluation. For example, the hardness of a bar can satisfactorily be determined by the use of the conventional grease testing procedure as described in ASTM method D-217. The hardness of a bar can thus be measured by the depth that a standard cone penetrates the sample, set at a temperature of 77° F., expressed in tenths of a millimeter. Any bar falling within the hardness range 2 to 20, more narrowly 5 to 15, is deemed satisfactory from the standpoint of hardness.

Another important property of a detergent bar is the solution rate of the active detergent component of the bar. As mentioned above, non-soap detergent bars are superior to soap in the respect that solubility and rates of solution are better in both hard and salt water. At any rate, a convenient way of measuring the solubility characteristics of detergent bar is by determining its loss in weight in grams per hand-wash employing ordinary tap water having a hardness of 50 p.p.m. and at a temperature of about 110° F., averaged from a number of hand-washings by different individuals. It has been determined that the wear rate of a satisfactory bar may range from about 0.7 to 1.5 g. per hand wash.

The bars employed in the following examples were

active detergent material in the conventional amounts, i.e., from about 5 to 65%, by weight.

In the following examples, hardness, wear rate, and water content were determined by the methods hereinbefore outlined. Ammonium sulfate content was determined by solutions of the anhydrous product bar material in isopropyl alcohol. All the sulfonate dissolves while the sulfate salt is insoluble. The insoluble matter is collected and dried by conventional gravimetric procedures.

As an example of the invention, calcium-ammonium alkylsulfonates are prepared from a mixture of alpha-olefins of about 8 to 20 carbon atoms and obtained by the cracking of petroleum wax, the average carbon content of the olefins being around 15. In the preparation of the detergent material, the sulfitation reaction above described is followed, using aqueous calcium hydroxide with boiling to displace the ammonium ion to the desired extent. After the addition of the calcium hydroxide, the product is dried as hereinabove described. The bar analyzes as follows:

|                                                                                     |      |
|-------------------------------------------------------------------------------------|------|
| Alkylsulfonate (calcium alkylsulfonate to ammonium alkylsulfonate, mol ratio 10:90) | 82.1 |
| Sulfate content                                                                     | 11.0 |
| Water, wt. percent                                                                  | 6.9  |
| Hardness                                                                            | 6.0  |
| Wear rate, g./wash                                                                  | 1.2  |

Using the same procedure as outlined above, a number of bars are prepared in which the active detergent material is a mixture of ammonium and sodium alkylsulfonates prepared from petroleum wax  $C_{10}$ - $C_{20}$  olefins. The data are tabulated below:

| Run No.                     | 1      | 2      | 3     | 4      | 5      | 6                 |
|-----------------------------|--------|--------|-------|--------|--------|-------------------|
| Mol ratio $Na^+ : NH_4^+$   | 0:100  | 15:85  | 25:75 | 50:50  | 64:38  | 100:0.            |
| Hardness                    | 150    | 16     | 12.5  | 7      | 6      | too hard to mold. |
| Sulfate, Wt. percent        | 13     | 12     | 15    | 12     | 11     | 11.               |
| Water, Wt. percent          | 6.5    | 2.4    | 4.8   | 4      | 6.9    | 3.                |
| Alkylsulfonate, Wt. percent | 80     | 85.6   | 81.4  | 84     | 82.2   | 85.               |
| Bar characteristics         | unsat. | satis. | good  | excel. | excel. | not formed.       |

obtained by drum-drying the detergent material to the desired water content into a film, after which the film was ground for homogeneity. The detergent material was then formed into a bar by molding in a conventional soap-bar mold. The bars weigh 2-3 ounces and have the approximate dimensions in inches of  $2\frac{1}{8} \times 2\frac{1}{8} \times \frac{3}{4}$ .

In the preparation of the sulfonate detergent material, aqueous ammonium bisulfite is added to the appropriate olefin material in aqueous alcohol solvent. Following the sulfitation reaction a de-oiling step is performed to remove unreacted hydrocarbons. These can be removed by extraction with a light hydrocarbon, e.g., pentane, or by dilution with water to effect phase formation of the oil and sulfonate followed by separation of the phases, as by decantation. An amount of appropriate base calculated to give the desired amount of mixed sulfonate salts is then added. The alcohol is next removed from the sulfonate layer by distillation. Heating is continued to remove more water until the water content of the product is about 20-25 weight percent of the mixture. At this point the product, a thick slurry which at about 100° C. still flows, is dropped upon a chilled roll, whereupon the product solidifies. The material is then chipped off the roll and air-dried in a conventional drier down to about 1-8 weight percent water, as determined for example by the Karl Fischer titration method.

The alkylsulfonate salts are now in condition for molding. If desired, at this stage there may be incorporated into the detergent material other ingredients for the purposes of improving the composition in such properties as odor, color and the like. Accordingly, known fillers, perfumes, dyes and the like can be incorporated with the

45 A bar is formed from ammonium and potassium primary n-alkylsulfonates derived from  $C_{10}$ - $C_{20}$  cracked wax olefins. It analyzes as follows:

|                                                                                   |     |
|-----------------------------------------------------------------------------------|-----|
| Alkylsulfonate (ammonium alkylsulfonate to potassium sulfonates, mol ratio 15:85) | 78  |
| Sulfate content                                                                   | 15  |
| Water, wt. percent                                                                | 5.0 |
| Hardness                                                                          | 7.0 |
| Wear rate, g./wash                                                                | 1.5 |

55 A satisfactory bar is prepared from ammonium and magnesium sulfonate, with the following characteristics:

|                                                                                           |     |
|-------------------------------------------------------------------------------------------|-----|
| N-alkylsulfonate (ammonium n-alkylsulfonate to magnesium n-alkylsulfonate, mol ratio 2:1) | 74  |
| Sulfate content                                                                           | 15  |
| Water, wt. percent                                                                        | 8   |
| Wear rate, g./wash                                                                        | 1.1 |

65 It is appreciated that alkylsulfonates, secondary as well as primary, as a class are broadly recognized to possess surface-active properties. The particular sulfonates herein described are believed to be unique in that they are readily formed in a satisfactory bar and have other desirable characteristics, such as, chemical stability and satisfactory rate of water solubility. As opposed to the primary alkylsulfonates of the present invention, the secondary sulfonates are unsatisfactory and cannot be formed into a bar. Similarly, other synthetic detergent materials such as those which form the great bulk of commercial detergent compositions, namely, the alkylaryl sulfonates and the alkyl sulfates cannot satisfactorily be formed into bars in accordance with the present invention.

70

tion. Thus, the alkyl sulfates are chemically unstable and hydrolyze readily in the presence of water, while the alkylaryl sulfonates on the other hand are too soluble and give a sticky feeling when employed in the form of a bar.

I claim:

1. A synthetic detergent bar consisting essentially of (1) ammonium n-alkyl sulfonate; (2) a second metal n-alkyl sulfonate to enable milling and molding in an amount of 10 to 75 weight percent based on (1) and (2); and (3) 1% to 10% water, by weight, based on (1) and (2); the alkyl groups in each of (1) and (2) being primary straight-chain radicals of about 8 to 20 carbon atoms and averaging 12 to 16 carbon atoms, the metal of said second metal n-alkyl sulfonate being selected from the group consisting of alkali and alkaline earth metals.

2. The synthetic detergent bar according to claim 1, wherein the second metal n-alkylsulfonate is sodium n-alkylsulfonate.

3. The synthetic detergent bar according to claim 1, wherein the second metal n-alkylsulfonate is selected from the group consisting of calcium and magnesium n-alkylsulfonates.

4. The synthetic detergent bar according to claim 1, wherein the water content is 5 to 8%.

References Cited in the file of this patent

5

UNITED STATES PATENTS

|           |         |               |
|-----------|---------|---------------|
| 2,374,187 | Flett   | Apr. 24, 1945 |
| 2,504,411 | Harman  | Apr. 18, 1950 |
| 2,813,078 | Vitalis | Nov. 12, 1957 |

FOREIGN PATENTS

|         |               |              |
|---------|---------------|--------------|
| 682,207 | Great Britain | Nov. 5, 1952 |
|---------|---------------|--------------|

OTHER REFERENCES

15 Mayo et al.: "The Peroxide Effect in the Addition of Reagents to Unsaturated Compounds and in Rearrangement Reactions, IV, The Reaction of Bisulfites With Unsaturated Compounds," Chemical Reviews, vol. 27 (October 1940), pp. 351-412.

20 Lelong et al.: "Electrical Conductances of Some Aqueous Solutions of Magnesium n-Alkane sulfonates," Jour. Amer. Chem. Soc., 73, 5411-14 (1951).

Lingafelter et al.: "Extent of Hydration of Some Crystalline Phases of Sodium 1-Alkanesulfonates," Jour. of Physical Chemistry, 57, 428-429 (April 1953).